

Patented Dec. 11, 1923.

1,477,511

# UNITED STATES PATENT OFFICE.

JAMES W. MARTIN, JR., OF CLENDENIN, WEST VIRGINIA, ASSIGNOR TO CARBIDE AND CARBON CHEMICALS CORPORATION, A CORPORATION OF NEW YORK.

## PROCESS OF MAKING CARBONBLACK.

No Drawing.

Application filed February 1, 1923. Serial No. 616,440.

To all whom it may concern:

Be it known that I, JAMES W. MARTIN, Jr., a citizen of the United States, residing at Clendenin, in the county of Kanawha and State of West Virginia, have invented certain new and useful Improvements in Processes of Making Carbonblack, of which the following is a specification.

The invention is a process of manufacturing carbon-black by the arrested combustion of hydrocarbons or mixtures thereof.

Carbon-black is extensively manufactured by burning natural gas in such a way that the carbon of the hydrocarbon molecules is not completely burned to gaseous products, the unburned carbon being deposited as a soot useful as a pigment and for other purposes. In such processes, combustion is arrested, as by bringing into the flame surfaces maintained at a low enough temperature to cool the products of combustion at an intermediate stage of the oxidizing reactions.

Burners and collecting surfaces of the widest variety have been proposed and used, but it has not been found possible to increase the yield of black above a certain maximum, nor to increase the tintorial power of the product beyond certain limits.

By the method of my invention, it is possible to produce from a given amount of material, a much larger amount of black than was obtainable by the process heretofore employed. The quality of the black thus produced is fully as good as the prior product and in many instances my product is of higher quality than the blacks now regarded as standard.

This improved result is obtained by preheating the gaseous hydrocarbon material before passing it to the burner. The optimum preheating temperature varies somewhat with different raw materials. In the case of a natural gas such as that largely employed in the West Virginia field for making carbon-black, a preheating temperature of about 400° C. is preferred. When the temperature to which the gas is preheated is below about 200° C., there is no important increase in the yield of carbon-black. With preheating temperatures between about 200° C. and about 300° C., there is a measurably increased yield. Above 300° C., the yield increases quite rapidly with the preheating temperature. Such hydrocarbon gases as have been in-

vestigated also show a limit which the preheating temperature should not exceed, because of the decomposition of the gas with deposition of carbon within the burner which results from excessive overheating. With some hydrocarbon mixtures the upper limit of preheating, fixed by this consideration, is as low as 500° C.

It is well known that gas is perceptibly preheated in its passage through burners of very many types, heat being conveyed from the flame to the burner, and thence to the gas within the burner by radiation or conduction, or even by convection. So far as I am aware, the amount of preheating which can take place in any burner heretofore used or proposed for the manufacture of carbon-black is entirely inadequate to give the advantageous effects obtainable with my invention.

The burners and other apparatus now employed are well adapted for use in connection with my process, and no complicated or expensive additions are required. It is sufficient merely to pass the gas, on its way to the burners, in such proximity to the flames, and for such a time, that it attains the desired temperature before reaching the burners. It is then burned and the black collected in accordance with any usual practice.

The process is applicable not only to natural gas but to fractions and concentrates therefrom, to other mixtures of gaseous hydrocarbons, and to single hydrocarbons such as ethane, propane, or butane as well.

In a particular instance, a material capable of giving only 0.7 pound of black per thousand cubic feet when not preheated, gave by my process 4.0 pounds of black per thousand cubic feet, the procedure remaining unchanged except for the provision of a preheating step.

This application is a continuation in part of the copending application Serial No. 596,871, filed by me Oct. 25, 1922.

I claim:

1. Process of making carbon black from hydrocarbon material aeriform under normal conditions of temperature and pressure, which comprises preheating said material to a temperature above 200° C. and then burning the material under conditions adapted to form carbon black.

2. Process of making carbon black from

- a gas mixture consisting of hydrocarbons normally present in natural gas, which comprises preheating said hydrocarbons to a temperature in excess of 200° C. and then 5 burning them under conditions adapted to form carbon black.
3. Process of making carbon black from natural gas of normal composition, which
- comprises preheating the gas to a temperature between 200° C. and 500° C., and then 10 burning the gas under conditions adapted to form carbon black.
4. Process according to claim 3 in which the preheating temperature is about 400° C.

In testimony whereof, I affix my signature.

JAMES W. MARTIN, JR.